

# UNITED STATES PATENT OFFICE.

REINHARD SCHMIEDEL, OF DRESDEN, GERMANY.

## LIQUID COMPOSITION TO BE USED IN THE MANUFACTURE OF FANCY STAINED PAPERS.

No. 882,916.

Specification of Letters Patent. Patented March 24, 1908.

Application filed May 19, 1904. Serial No. 208,660.

To all whom it may concern:

Be it known that I, REINHARD SCHMIEDEL, a subject of the King of Saxony, and resident of Dresden, Stephanienstrasse 95, Kingdom 5 of Saxony, Germany, have invented a new and useful Liquid Composition to be Used in the Manufacture of Fancy Stained Papers, of which the following is a specification.

In the manufacture of fancy stained papers 10 the pattern of which corresponds to the primary paint applied to the paper and comes out by a darker tone only, it was necessary heretofore to use a paint to produce such darker tone. In most cases many attempts 15 or tests were necessary to secure the tone suitable for the purpose, such attempts or tests causing a great waste of time, especially if the paint must be produced by mixing.

The composition which is the subject of 20 the present invention has for its object to dispense with the use of paint in the production of patterns of the kind mentioned above, to economize or spare time and also to secure an image of a more brilliant and 25 clearer color.

The composition can be used for stained paper of any kind, no matter whether its surface is dead or brilliant, pressed or smooth. Dead paper does not become brilliant by its 30 use and a brilliant one does not become dead or subdued and the smooth and pressed surface of the paper is maintained and the brilliancy of glazed, bronze or mica papers is not altered.

The composition which is in liquid form is 35 used in combination with or during applying the pattern to the paper provided with the primary color, such applying or covering being effected by a mold, brush or any other suitable means. This liquid or mixture con-

sists of the solution of a moist colorless substance or agent, which after evaporating of the solvent adheres as a precipitate to the fibers of the paper and acts on the primary paint adhering to such paper by darkening.

45 The composition consists mainly of a diluted and easily drying mixture at the ordinary temperature of an agglutinant soluble in water or alcohol with soap, oil, glycerin, alcohol and water. The said agglutinant, 50 may be glue, gumarabic, dextrin or the like.

The denaturation of the alcohol may be effected by wood-alcohol, shellac, camphor, turpentine, formalin, animal-oil, benzene, petroleum-benzin, castor-oil, soda-lye or various salts.

According to the value or importance attached more or less to the ardor, clearness and beauty of the color-tones produced by means of the present invention, the liquid used consists either of a very volatile solvent, as alcohol, benzene, carbon tetrachlorid and the like and a resin soluble in such agents, as colophony, and the like or a solvent evaporating not so quickly. The finally prepared mixture is neutralized by acids.

65 I have found as well suitable for the purpose the following mixtures which produce the tones to be obtained in all primary colors.

|    |               |    |
|----|---------------|----|
| 30 | grams glue,   | 70 |
| 40 | " gum-arabic, |    |
| 10 | " glycerin,   |    |
| 40 | " dextrin,    |    |
| 40 | " alcohol,    |    |
| 30 | " soap,       |    |
| 60 | " water,      | 75 |

or

|    |                |    |
|----|----------------|----|
| 30 | grams dextrin, |    |
| 30 | " glue,        |    |
| 30 | " tannin,      | 80 |
| 30 | " alcohol,     |    |
| 30 | " soap,        |    |
| 30 | " water,       |    |
| 30 | " glycerin,    |    |

or

|    |                    |    |
|----|--------------------|----|
| 50 | grams gum-juniper, |    |
| 20 | " glue,            |    |
| 10 | " glycerin,        |    |
| 30 | " soap,            |    |
| 10 | " turkey-red oil,  | 90 |
| 50 | " alcohol,         |    |
| 80 | " water            |    |

or

|    |                                                    |     |
|----|----------------------------------------------------|-----|
| 30 | grams fish-glue,                                   |     |
| 20 | " tannin,                                          | 95  |
| 30 | " glue,                                            |     |
| 30 | " resin from fruit-trees,                          |     |
| 50 | " soap,                                            |     |
| 50 | " alcohol with the addition of 25 grams colophony, | 100 |
| 80 | " water                                            |     |

or

|    |                   |     |
|----|-------------------|-----|
| 50 | grams gum-dragon, |     |
| 30 | " casein,         |     |
| 30 | " gum-arabic,     | 105 |
| 50 | " alcohol,        |     |
| 50 | " dextrin,        |     |
| 30 | " soap,           |     |
| 70 | " water,          |     |
| 50 | " oil.            | 110 |

According to the primary - tone to be printed and to the brighter or darker color tone to be produced on it, the composition mentioned above may be of a higher or lower 5 degree of strength which may be obtained by using the agglutinative substances, as dextrin, glue, resin and the like in greater quantities, or the addition of water may be a greater one if the tone to be produced shall 10 be of greater or smaller brilliancy.

By the use of the object of the present invention it is possible to obtain, even with the employment of the clearest warmest colors for instance turkey-red, cherry-red etc. with 15 the paint a warm tone-shadow, which cannot be obtained by means of other processes. Furthermore in stained patterns printed on paper or by lithography and in another suitable mechanical manner it is possible to produce each tone-shadow within the tones 20 created by the transfer of an effect in each

finished image, as for instance in flowers the primary colors red, blue, green, yellow can be shadowed simultaneously and at once with the use of the paints according to the 25 present invention.

What I claim is:

A liquid composition to be used in the manufacture of stained paper consisting of a diluted and easily drying mixture of an ag- 30 glutinant soluble in water or alcohol with soap, oil, glycerin, alcohol and water, substantially as herein described.

In testimony, that I claim the foregoing as my invention, I have signed my name in 35 presence of two witnesses, this seventh day of May, 1904.

REINHARD SCHMIEDEL.

Witnesses:

OTTO H. KNOOP,  
ERNST C. MEYER.